

March 31, 1959

L. MUSICANT

2,880,326

NEUTRON DETECTOR

Filed Oct. 25, 1954



LOUIS MUSICANT  
INVENTOR

BY *Ralph E. Bitner*

ATTORNEY

1

2,880,326

**NEUTRON DETECTOR**

Louis Musicant, Irvington, N.J., assignor to National Radiac, Inc., Newark, N.J., a corporation of New Jersey

Application October 25, 1954, Serial No. 464,256

8 Claims. (Cl. 250—71.5)

This invention relates to neutron detectors and has particular reference to polymers of boron mixed with fluorescent substances used in conjunction with a light sensitive element.

The detection of neutrons has been accomplished in the past in various ways, such as, the employing of scintillation crystals of lithium iodide mixed with various fluorescent powders, Geiger counters having a boron compound on the inner surface of the glass envelope or filled with boron trifluoride gas, and liquid scintillators. Each of these detectors has inherent disadvantages which prohibit their use except as laboratory instruments. The lithium iodide crystals are very expensive and are difficult to grow. Geiger tubes are fragile and with a boron compound within the envelope have a short operating life. The liquid scintillators are unwieldy and have a low efficiency.

In order to overcome the above disadvantages a number of boron ester polymers have been prepared containing fluorescent substances which are cheap and easy to manufacture. They can be protected against mechanical shock and are efficient neutron detectors. One such polymer is polyalcohol borate dispersed with powdered zinc sulfide. The boron content of this detector has been found to be between 23 and 24 percent by actual analysis and this high percentage of boron accounts for the relatively high efficiency. Other detectors such as polyethylene glycol borate will be described hereinafter.

One of the objects of this invention is to provide an improved neutron detector which avoids one or more of the disadvantages and limitations of prior art detectors.

Another object of the invention is to reduce the cost of neutron detectors.

Another object of the invention is to eliminate the dead time which is always present in Geiger counters.

Another object of the invention is to increase the portability and ruggedness of neutron counters so they may be taken into the field and transported without fear of failure.

One feature of the invention includes the mixture of a fluorescent powder and a boron ester polymer. This mixture is translucent and produces light flashes when bombarded with neutrons.

Another feature of the invention includes a light sensitive element mounted adjacent to the above described mixture and enclosed in a chamber which permits neutrons to pass but which excludes light and other types of penetrating radiation.

For a better understanding of the present invention, together with other and further objects thereof, reference is made to the following description taken in connection with the accompanying drawing.

The single figure is a block diagram showing the container in section. A container 10 is provided for supporting a plastic block 11 and a photoelectric tube 12. The container walls may be made of lead or steel sheet in order to shield the plastic block from light and other forms of penetrating radiation such as alpha, beta,

2

gamma, or X-rays. If it is known that such latter radiation is absent the only shield required is a light shield.

A photoelectric cell 12 is indicated in the drawing because it has been found that such a device is more sensitive than any other form of light sensitive device. However, any form of transducer which converts light energy to electric energy may be used in this arrangement.

The electrical variations provided by the photocell 12 are transferred over conductors which pass through light-tight insulators 13 and are connected to an amplifier 14 if necessary. A power supply 15 is connected to the amplifier and also supplies the photocell with operating voltage. An indicator 16 is connected to the amplifier output and shows the extent of the light generated by the plastic block 11 and is therefore a measure of the number of neutrons which strike the block.

The plastic block 11 must have a high percentage of boron atoms in its molecular structure because the boron is the active indicator which determines the presence of neutrons. When a neutron strikes a boron atom an alpha particle is emitted and the alpha particle is detected by its action on some fluorescent substance such as zinc sulphide which is dispersed homogeneously in the block. The block should also be transparent or reasonably translucent so that thick blocks can be used, the light flashes from the portion farthest from the light sensitive element thereby producing the same effect as near by flashes.

30 A neutron detector having the above listed characteristics can be made as follows: Forty grams of boric acid and ten grams of ethylene glycol are mixed together and heated to about 200 degrees centigrade until moisture is no longer evolved. The final product weighs 32.4 grams and contains 21.6 percent boron. By increasing the proportion of boric acid to ethylene glycol, the boron content can be increased to 24 percent. To the above liquid is now added 64.8 grams of activated zinc sulfide in powdered form having a particle size within the range of five to ten microns. One such grade of zinc sulfide is known commercially as "du Pont 2B1-ZnS." This mixture is stirred thoroughly to obtain uniform dispersion and the mixture is cooled to room temperature. The resultant product may be stored in a desiccator to protect it from the moisture in the atmosphere or it may be processed immediately to form plates or blocks. The molding may be done by placing the material in a prepared mold in a hydraulic press. The mold is heated to a temperature of about 115 degrees centigrade and subjected to a pressure of 5,000 to 10,000 pounds per square inch. The result is a translucent block of polyethylene glycol borate having evenly dispersed zinc sulfide and more than 20 percent boron content.

Another formulation is produced as follows: Five grams trimethylol ethane and fifteen grams of boric acid are heated together gently in a test tube until all the moisture is driven out. The recovered plastic is poly-trimethylol borate and weighs 14.6 grams. To this is added 29.2 grams of powdered zinc sulfide. The mixture is heated to about 190 degrees centigrade and stirred to produce a homogeneous mass. The resulting mixture can be molded in the same manner as the polyethylene glycol borate mixture.

65 Neutron detecting phosphors can also be made from other polyalcohols such as propylene glycol, sorbitol, glycerin, etc. The borate zinc sulfide mixtures are prepared in the same manner as the examples described above.

The above described phosphors have an absolute efficiency for thermal neutrons of 20 percent when the phosphor plate is  $\frac{1}{16}$  inch thick.

70 Two neutron phosphors have been described and their

use illustrated. From the above description it will be obvious that other similar products can be made without departing from the field of the invention which should be limited only by the scope of the appended claims.

I claim:

1. A neutron detector comprising a transparent solid homogeneous mixture of a fluorescent substance and a boron ester polymer, said mixture containing at least 20 percent of boron by weight.

2. A neutron detector which produces light when bombarded by neutrons comprising a transparent solid homogeneous mixture of a fluorescent substance and a boron ester polymer, said mixture containing at least 20 percent of boron by weight.

3. A neutron detector as set forth in claim 2 wherein said fluorescent substance emits flashes of light when bombarded by alpha particles.

4. A neutron detector which produces light when bombarded by neutrons comprising a solid transparent homogeneous mixture of a fluorescent substance and

polyethylene glycol borate, said mixture containing at least 20 percent of boron by weight.

5. A neutron detector as set forth in claim 4 wherein said fluorescent substance is zinc sulfide.

6. A neutron detector as set forth in claim 2 wherein said boron ester polymer is polytrimethylol borate.

7. A neutron detector as set forth in claim 2 wherein said solid mixture is mounted adjacent to a light sensitive element.

10 8. A neutron detector as set forth in claim 7 wherein said light sensitive element converts light energy to electrical energy and includes conductive connections to an electrical indicating means.

15

**References Cited in the file of this patent**

"Two Liquid Scintillation Neutron Detectors," by Muehlhause and Thomas, from Nucleonics, vol. 11, No. 1, January 1953, pp. 44, 45.

20 "A Fast Neutron Scintillator," by Emmerich, from the Review of Scientific Instruments, vol. 25, No. 1, January 1954, pp. 69, 70.